

Oct. 23, 1945.

R. F. BRENNER

2,387,561

METHOD OF TREATING THE ROCK, APLITE

Filed March 26, 1943

7 Sheets-Sheet 1



Fig. 1

INVENTOR.  
Ralph F. Brenner.

BY  
*Cabell, Mahaney & Miller*  
ATTORNEYS

Oct. 23, 1945.

R. F. BRENNER

2,387,561

METHOD OF TREATING THE ROCK, APLITE

Filed March 26, 1943 7 Sheets-Sheet 2



Fig. 2

INVENTOR.  
Ralph F. Brenner.

BY  
*Cubitt, Whitney & Miller*  
ATTORNEYS

Oct. 23, 1945.

R. F. BRENNER

**2,387,561**

## METHOD OF TREATING THE ROCK, APLITE

Filed March 26, 1943

7 Sheets-Sheet 3



Fig. 3

PERCENTAGE INCREASE IN GRINDABILITY DUE TO CALCINATION

INVENTOR.  
Ralph F. Brenner

BY  
*Carbett, Mahoney & Miller*  
ATTORNEYS

Oct. 23, 1945.

R. F. BRENNER

2,387,561

METHOD OF TREATING THE ROCK, APLITE

Filed March 26, 1943

7 Sheets-Sheet 4



Fig. 4

INVENTOR.  
Ralph F. Brenner

BY  
*Curtiss, Mohrway & Miller*  
ATTORNEYS

Oct. 23, 1945.

R. F. BRENNER

2,387,561

METHOD OF TREATING THE ROCK, APLITE

Filed March 26, 1943

7 Sheets-Sheet 5



Fig. 5

INVENTOR  
Ralph F. Brenner

BY  
*Curtiss, Malony & Miller*  
ATTORNEYS

Oct. 23, 1945.

R. F. BRENNER

2,387,561

METHOD OF TREATING THE ROCK, APLITE

Filed March 26, 1943

7 Sheets-Sheet 6



Fig. 6

PER CENT INCREASE IN MINUS 16 PLUS 100-MESH PRODUCT OF GRINDABILITY  
TESTS DUE TO CALCINATION-UNCALCINED PRODUCTS BEING CONSIDERED AS 100 PER CENT

INVENTOR.  
Ralph F. Brenner.

BY

*Curtis, Molony & Miller*  
ATTORNEYS

Oct. 23, 1945.

R. F. BRENNER

2,387,561

METHOD OF TREATING THE ROCK, APLITE

Filed March 26, 1943

7 Sheets-Sheet 7



Fig. 7



Fig. 8



Fig. 9



Fig. 10



Fig. 11



Fig. 12



Fig. 13



Fig. 14



Fig. 15



Fig. 16

INVENTOR.  
Ralph F. Brenner

BY

Corbett, Mahaney & Miller  
ATTORNEYS

## UNITED STATES PATENT OFFICE

2,387,561

## METHOD OF TREATING THE ROCK, APLITE

Ralph F. Brenner, Lancaster, Ohio, assignor to  
 Dominion Minerals, Incorporated, Washington,  
 D. C., a corporation of Virginia

Application March 26, 1943, Serial No. 480,641

2 Claims. (Cl. 241—32)

My invention relates to a method of treating the rock, aplite. It has to do, more particularly, with a method of treating aplite preparatory to grinding.

This application is a continuation-in-part of my copending application Serial No. 397,599, filed June 11, 1941, now Patent 2,368,194, issued January 30, 1945.

Aplite is a rather fine-grained granitic rock of equi-granular structure consisting chiefly of an intergrowth of quartz and feldspar with possibly some muscovite mica and usually occurs in dykes. A form of it, commercially mined chiefly in Virginia, has the following approximate chemical composition:

|                                                   | Per cent |
|---------------------------------------------------|----------|
| Albite (Al 90, An 10) .....                       | 55       |
| Zoisite .....                                     | 22       |
| Sericite .....                                    | 13       |
| Microcline .....                                  | 5        |
| Quartz .....                                      | 3        |
| Titanite, garnet, apatite and clino-zoisite ..... | 2        |

At the present time, considerable difficulty is encountered in grinding the rock aplite due to its excessive hardness, the lack of cleavage, and the tendency to produce an excessive amount of fines during grinding. In grinding aplite at the present time, a large amount of fines, finer than 200 mesh, are produced because of the nature of the grinding action required to reduce the extremely hard lumps into grains of suitable size. Due to the nature of these fines, a large percentage of this material is waste material. Also, because of the extreme hardness and lack of cleavage of the aplite, it is necessary to have very rugged and wear-resistant grinding equipment, which is expensive, and still excessive wear occurs.

As indicated in Patent No. 2,304,440, issued to Ralph F. Brenner and Roger D. Dubble, on December 8, 1942, the rock aplite has iron in combined form therein, and it is very desirable to reduce this iron content in order to make the aplite suitable for use in ceramic mixtures, such as in glass batches, or for similar uses.

One of the objects of my invention is to treat the rock aplite before grinding in such a manner that its resistance to grinding will be reduced, due to a change in physical structure.

Another object of my invention is to treat the rock aplite before grinding in such a manner that grinding will not only be facilitated but also subsequent treatment to remove the iron content will be facilitated.

Another object of my invention is to treat the rock aplite before grinding in such a manner that excessive wear on the grinding equipment will be reduced to a minimum.

Another object of my invention is to treat the rock aplite in such a manner before grinding that its resistance to grinding will be greatly reduced and its physical structure changed so that the grinding operation required to reduce the lumps of aplite to suitable grain size will not be of such a nature as to produce a high percentage of fines.

Another object of my invention is to provide a complete and efficient process for treating the rock aplite, as mined, to reduce it to the proper grain size and to reduce the iron content thereof.

The rock aplite, as mined, usually consists of lumps of various sizes. As previously indicated, it has been very difficult to grind these lumps in order to produce grains of the proper size. I have found that if the aplite is subjected to a proper calcining or heat-treating operation before grinding, grinding is facilitated. I have discovered that for this purpose it is desirable to calcine or heat-treat the aplite at a temperature in excess of 1000° F. and up to the fusion point of the aplite, which usually is about 2237° F. The most effective and preferred range of calcining temperatures is between 1650 and 2000° F. The time of heating will depend upon the size of the lumps of the aplite. It is merely necessary to heat the aplite for a period sufficient for the heat to penetrate completely into the interior of the lumps. After the aplite is subjected to this heat-treatment, it is cooled in air or water-quenched or sprayed. I prefer to either water-

40 quench or spray the aplite.

Although I do not wish to be limited to any particular theory, the calcining or heat-treating operation apparently changes the physical structure of the aplite, causing permanent expansion or dilatation thereof and fracturing preferentially along the grain boundaries thereof. This apparently is the reason for the improvement in the grindability of the aplite and for the production of a greater percentage of ground material of the desired screen size.

In order to establish the grinding characteristics of aplite and to establish the temperature at which calcination should be carried out prior to grinding, certain tests were made. Similar tests were made on other materials, such as soda feldspar, potash feldspar, and quartz, to show that the results obtained by calcining aplite within the proper temperature range are caused by properties characteristic of aplite and not of the individual minerals contained in the aplite.

The accompanying drawings will aid in understanding these tests and the results obtained. In these drawings:

Figure 1 is a diagram showing expansion and cooling curves for aplite, soda feldspar, potash feldspar and quartz, heated at temperatures within the range, room temperature to 2000° F.

Figure 2 is a diagram showing curves for grindability indices plotted against calcination temperature obtained from various calcined samples of aplite, soda feldspar, potash feldspar and quartz.

Figure 3 is a diagram showing curves which indicate the percentage increase in grindability, owing to calcination, of calcined samples of aplite, soda feldspar, potash feldspar, and quartz.

Figure 4 is a diagram showing curves in which the percentage of plus 16-mesh material is plotted against temperature for the calcined and uncalcined samples of aplite, soda feldspar, potash feldspar and quartz.

Figure 5 is a diagram showing curves in which the percentage of minus 16 plus 100-mesh material is plotted against temperature for the calcined and uncalcined samples of aplite, soda feldspar, potash feldspar and quartz.

Figure 6 is a view wherein the curves indicate the percentage increase in minus 16 plus 100-mesh material plotted against temperature for the calcined and uncalcined samples of aplite, soda feldspar, potash feldspar and quartz.

Figure 7 is a reproduction of a photomicrograph of an uncalcined sample of aplite taken under a polarizing microscope at 10 magnifications without crossed nicols.

Figure 8 is a photomicrograph at 10 magnifications which is the same field as Figure 7 and which was photographed with crossed nicols.

Figure 9 is a crossed nicols photomicrograph at 10 magnifications of a sample of aplite calcined at 1000° Fahrenheit.

Figure 10 is a similar view of a sample of aplite calcined at 1300° Fahrenheit.

Figure 11 is a similar view of a sample of aplite calcined at 1500° Fahrenheit.

Figure 12 is a similar view of a sample of aplite calcined at 1650° Fahrenheit.

Figure 13 is a similar view of a sample of aplite calcined at 1800° Fahrenheit.

Figure 14 is a similar view of a sample of aplite calcined at 2000° Fahrenheit.

Figure 15 is a similar view of a sample of aplite calcined at 2150° Fahrenheit.

Figure 16 is a photomicrograph at 10 magnifi-

cations which is the same field as Figure 15 but which was photographed without crossed nicols.

To establish the grinding characteristics of the materials in question before calcination and after they had been calcined at various significant temperatures, it was decided to use the "Grindability index" method developed by Bond and Maxson\* as a means of showing changes in grinding characteristics owing to calcination.

10 In addition to tests on aplite, in this work, the effect of calcination on grindability was studied for soda feldspar (albite), potash feldspar (microcline), and quartz. The reason for including soda feldspar, potash, feldspar and quartz in this 15 investigation is that they are major constituents of aplite rock and it was desired to show that in the particular temperature range where calcination renders aplite least resistant to grinding, the effect is due to some change which is inherent 20 in the makeup of aplite and that cannot be accounted for by the physical changes that take place in soda feldspar, potash feldspar and quartz.

The samples of aplite, soda feldspar, potash 25 feldspar and quartz used in this investigation were received in lumps, some as coarse as 10 inches. The largest lumps were sledged down to crusher size and then each material was carefully stage crushed to minus  $\frac{1}{4}$  inch.

30 Table 1 which follows gives the chemical composition of the aplite, soda feldspar, potash feldspar and quartz samples.

Table 1.—Chemical composition of aplite, soda feldspar, potash feldspar, and quartz samples

|    | Elements                                | Aplite | Soda feldspar | Potash feldspar | Quartz |
|----|-----------------------------------------|--------|---------------|-----------------|--------|
| 40 | SiO <sub>2</sub> ..... percent          | 60.25  | 64.00         | 64.80           | 96.8   |
|    | Fe <sub>2</sub> O <sub>3</sub> ..... do | 0.60   | 0.40          | 0.02            | (1)    |
|    | Al <sub>2</sub> O <sub>3</sub> ..... do | 24.25  | 22.10         | 22.00           | -----  |
|    | CaO..... do                             | 6.60   | 2.90          | -----           | -----  |
|    | MgO..... do                             | -----  | 0.21          | -----           | -----  |
|    | Na <sub>2</sub> O..... do               | 5.75   | 7.70          | 2.27            | -----  |
|    | K <sub>2</sub> O..... do                | 3.00   | 0.60          | 10.46           | -----  |
| 45 | Ignition loss.....                      | 0.45   | 0.11          | 0.08            | 0.48   |

<sup>1</sup> Blank spaces indicate that no determination was made.

<sup>2</sup> Ignition gain.

The mineralogical composition of this same 55 aplite rock has been given previously. The soda feldspar was optically identified as albite (Al 90, An 10), the potash feldspar as microcline and the quartz as alpha quartz.

In order to determine whether the materials under consideration passed through inversion or transition points on heating and to establish the 60 temperatures at which calcination should be carried out prior to grinding, dilatometer tests were made. The tests were made in a Rockwell-Bristol, model A-116, dilatometer machine. The Rockwell-Bristol dilatometer is an instrument that measures dilatation or elongation with increase in temperature and plots temperature-dilatation and time-dilatation curves.

Figure 1 presents the temperature dilatation data obtained in these tests. This figure was prepared by plotting on rectangular coordinates, inches of elongation as ordinate and temperature in degrees Fahrenheit as abscissa. These four specimens were all dilatometrically treated in the same manner and presenting them in one figure shows the relative expansion of aplite, soda feldspar, potash feldspar and quartz in the range

\* A. I. M. E. Milling Methods, 1934, pages 130 to 145, and A. I. M. E. Milling Methods, 1939, pages 296 to 300.

room temperature to 2000° Fahrenheit and the contraction as the specimens were allowed to cool to room temperature.

The curve for soda feldspar shows that its elongation is quite uniform until a temperature of 1650° Fahrenheit is reached, where a transition point occurs and the elongation increases rapidly to six times its previous rate. When it reaches 1800° Fahrenheit, the elongation is slowed down and at 1900° Fahrenheit shrinkage begins. The cooling curve is uniform and shows that soda feldspar does not pass through a transition point on cooling. The vertical displacement between the beginning of the heating curve and the end of the cooling curve shows that the permanent dimensional change is slight.

The curves for potash feldspar show that it has uniform elongation with heating and that it contracts to practically its original length upon cooling. The uniformity of these curves indicate that potash feldspar does not pass through a transition point in the temperature range studied.

The curve for quartz shows that it has a much more rapid elongation than either potash feldspar or soda feldspar and that this elongation is uniform until a temperature of about 1100° Fahrenheit is reached, where the curve flattens off with practically no further elongation up to 1800° Fahrenheit followed by slight shrinkage up to 2000° Fahrenheit. The change in the slope of the quartz curve at 1100° Fahrenheit indicates an inversion point and a change from alpha to beta quartz. It is significant that the cooling curve passes through this same inversion point, showing that the change is reversible and a permanent dimensional change does not persist.

The fact that the specimens of soda feldspar, potash feldspar, and quartz return very nearly to their original lengths warrants the conclusion that their permanent expansion caused by heating is slight.

The aplite expansion curve shows that the elongation is uniform until a temperature of 1650° Fahrenheit is reached where a slight increase in temperature results in phenomenal elongation. The rate of increase between 1650° Fahrenheit and 1850° Fahrenheit is 5.3 times as great as the rate between room temperature and 1650° Fahrenheit. This indicates a marked transition point, and it is possible that had the dilatometer furnace been held at a constant temperature of about 1650° Fahrenheit, most of this elongation would have taken place without further increase in temperature. At 1850° Fahrenheit the curve assumes a rate approximately equal to that between room temperature and 1650° Fahrenheit and maintains this rate to 2000° Fahrenheit. The expansion curve described for aplite is similar to that described earlier for soda feldspar but the total expansion of the aplite is three times greater.

The cooling curve for aplite does not parallel the heating curve for there is no reverse transition at 1650° Fahrenheit and the total contraction is only one third of the expansion. In marked contrast to the curves for soda feldspar, potash feldspar, and quartz the aplite retains a large permanent deformation.

Two other dilatometer tests were made on aplite the curves for which are not shown in Figure 3. In one of these tests the maximum temperature employed was 1400° Fahrenheit, that is below the aplite transition temperature. The cooling curve came back to the starting point

showing that when aplite is heated below its transition point, the operation is reversible. In the other test, the aplite was heated to 2000° Fahrenheit, then cooled slowly and heated a second time to 2000° Fahrenheit and cooled. The curves for this test showed that the curves for the second heating and cooling followed the first cooling curve, starting and ending at the same point. This is added proof that aplite undergoes a permanent dimensional change when heated to 1650° Fahrenheit, but that when expanded aplite is again heated, only reversible changes occur.

#### Calcination tests

In view of the facts presented in Figure 1, samples of each of the materials were calcined at the following temperatures: 1000° Fahrenheit, which is below the transition point of any of the minerals; 1300° Fahrenheit, which is above the inversion point for quartz; 1500° Fahrenheit, which is below the transition point in aplite and soda feldspar; 1650° Fahrenheit, which is at the transition point for aplite and soda feldspar; 1800° Fahrenheit, which is near the middle of the aplite transition zone; and 2000° Fahrenheit, which is at the end of the aplite transition zone and the reversing point for quartz. Another temperature was desired in order that the maximum limit or temperature range in which calcining is effective would be established. This was obtained by observing the lowest calcining temperature at which softening of the aplite took place. Although the fusion point of aplite is said to be 2237° Fahrenheit, it becomes soft at 2150° Fahrenheit, so the latter temperature was chosen as the upper limit for the calcining tests.

In the furnace used in calcining these samples, the samples were brought to the desired temperature and held there for fifteen minutes in a neutral atmosphere after which the calcined material was removed from the furnace and allowed to cool in air.

Table 2 which follows shows the average temperatures maintained for the 15-minute calcination periods. Screen analyses were made of each of the 27 test samples calcined as above. These samples were then used in the grindability tests now to be described.

Table 2.—Average temperatures in degrees Fahrenheit for fifteen minute calcination periods

| Desired calcination temperature | Aplite | Soda feldspar | Potash feldspar | Quartz |
|---------------------------------|--------|---------------|-----------------|--------|
| 1,000                           | 1,020  | 1,020         | 1,030           | 960    |
| 1,300                           | 1,324  | 1,256         | 1,260           |        |
| 1,500                           | 1,483  | 1,502         | 1,505           | 1,518  |
| 1,650                           | 1,688  | 1,660         | 1,638           | 1,645  |
| 1,800                           | 1,780  | 1,798         | 1,781           | 1,763  |
| 2,000                           | 1,974  | 2,006         | 1,980           | 1,990  |
| 2,150                           | 2,121  | 2,140         | 2,162           | 2,133  |

#### Grindability tests

Samples of the various materials were used in a series of grindability tests based on the method of Bond and Maxson to determine the relative grindabilities of the four uncalcined materials and to determine the effect of calcination upon their grinding characteristics.

The grinding characteristics of the samples were shown by the grindability index which is the number of grams of finished material through a given mesh produced per revolution of a ball

mill. In this work, 16 mesh was taken as the limiting size.

The grindability index figure represents the relative ease or difficulty in grinding a sample to a particular mesh, rather than the relative hardness of the material itself. The grindability indices obtained from the uncalcined samples and the various treated samples of aplite, soda feldspar, potash feldspar, and quartz are given in Table 3 which follows.

Table 3.—Grindability indices of calcined and uncalcined samples and percentage increase in grindability index owing to calcination

| Material        | Calcination temperature, degrees F. | Grindability index, grams per revolution | Percentage increase in grindability index owing to calcination |
|-----------------|-------------------------------------|------------------------------------------|----------------------------------------------------------------|
| Aplite          | ( <sup>1</sup> )                    | 2.104                                    | 100                                                            |
| Do              | 1,000                               | 2.660                                    | 126                                                            |
| Do              | 1,300                               | 3.650                                    | 173                                                            |
| Do              | 1,500                               | 3.406                                    | 162                                                            |
| Do              | 1,650                               | 10.380                                   | 493                                                            |
| Do              | 1,800                               | 9.934                                    | 472                                                            |
| Do              | 2,000                               | 10.313                                   | 490                                                            |
| Do              | 2,150                               | 5.248                                    | 249                                                            |
| Soda feldspar   | ( <sup>1</sup> )                    | 4.617                                    | 100                                                            |
| Do              | 1,000                               | 4.719                                    | 102                                                            |
| Do              | 1,500                               | 6.594                                    | 143                                                            |
| Do              | 1,650                               | 8.961                                    | 194                                                            |
| Do              | 1,800                               | 9.001                                    | 195                                                            |
| Do              | 2,000                               | 8.480                                    | 184                                                            |
| Do              | 2,150                               | 5.588                                    | 120                                                            |
| Potash feldspar | ( <sup>1</sup> )                    | 5.060                                    | 100                                                            |
| Do              | 1,000                               | 5.174                                    | 102                                                            |
| Do              | 1,300                               | 5.352                                    | 106                                                            |
| Do              | 1,500                               | 5.799                                    | 115                                                            |
| Do              | 1,650                               | 6.249                                    | 123                                                            |
| Do              | 1,800                               | 7.295                                    | 144                                                            |
| Do              | 2,000                               | 7.149                                    | 141                                                            |
| Do              | 2,150                               | 5.930                                    | 117                                                            |
| Quartz          | ( <sup>1</sup> )                    | 3.224                                    | 110                                                            |
| Do              | 1,000                               | 3.362                                    | 104                                                            |
| Do              | 1,300                               | 4.092                                    | 127                                                            |
| Do              | 1,500                               | 4.450                                    | 138                                                            |
| Do              | 1,650                               | 4.420                                    | 137                                                            |
| Do              | 1,800                               | 4.326                                    | 134                                                            |
| Do              | 2,000                               | 4.330                                    | 134                                                            |
| Do              | 2,150                               | 5.139                                    | 159                                                            |

<sup>1</sup> Uncalcined.

The same results are presented in graphical form in Figure 2 where grindability index is plotted against calcination temperatures. This figure shows that in an uncalcined condition aplite is the hardest to grind, followed in order by quartz, soda feldspar, and potash feldspar. When calcined at 1000° Fahrenheit, aplite alone shows a slight increase in grindability. Between 1000° Fahrenheit and 1300° Fahrenheit there is an increase in the grindability of the quartz, agreeing with the dilatometer data which showed

the inversion from alpha to beta quartz at about 1100° Fahrenheit. In the same temperature range the aplite curve practically parallels the quartz curve, and there is very little improvement in the grindability of potash feldspar. There was not sufficient soda feldspar to make calcination tests at all temperatures, and a test at a temperature of 1300° Fahrenheit was omitted.

At 1650° Fahrenheit, there is an increase in the grindability of all of the materials except quartz which remains practically constant through the range 1500° to 2000° Fahrenheit. This is conclusive evidence that heating quartz beyond 1500° Fahrenheit does not materially improve its grindability, and it cannot be responsible for the increased grindability of aplite between 1650° and 2000° Fahrenheit, which is unusually marked and agrees with the transition temperature at which permanent deformation takes place as shown by the dilatometer data. From Figure 2 one might be led to believe that the two feldspars were responsible for the increased grindability of aplite in this temperature range. In order to show more clearly the differences in the grinding characteristics, Figure 3 is given.

In Figure 3, the percentage increase in grindability is plotted against calcining temperature. This figure shows that in comparison with the uncalcined materials, the grindability of aplite calcined between 1650° and 2000° Fahrenheit is increased 500 per cent. For the same calcination temperature range, the grindability of soda feldspar is increased only 200 per cent, and the grindability of quartz and potash feldspar, only 150 per cent. Figure 3 shows that the percentage increase in grindability is so much greater for aplite than for any of the other materials that they cannot account for this characteristic in aplite.

Referring again to the data in Figure 2, it shows that although aplite was the hardest to grind in the uncalcined condition, it was the easiest to grind after calcination in the range of 1650° to 2000° Fahrenheit.

#### 45 Size composition of grindability samples

It may be thought that calcination alone without grinding would account for an appreciable increase in the fines found in the grindability samples. That this is not the case is shown in Tables 4, 5, 6 and 7, which follow, which give the screen size distribution of products after calcination but prior to grinding for aplite, soda feldspar, potash feldspar and quartz, respectively.

Table 4.—Size distribution of aplite samples after calcination but prior to grinding

| Mesh size | Uncalcined |              | 1000° F. |              | 1300° F. |              | 1500° F. |              | 1650° F. |              | 1800° F. |              | 2000° F. |              | 2150° F. |              |
|-----------|------------|--------------|----------|--------------|----------|--------------|----------|--------------|----------|--------------|----------|--------------|----------|--------------|----------|--------------|
|           | Wt. %      | Cumul. wt. % | Wt. %    | Cumul. wt. % | Wt. %    | Cumul. wt. % | Wt. %    | Cumul. wt. % | Wt. %    | Cumul. wt. % | Wt. %    | Cumul. wt. % | Wt. %    | Cumul. wt. % | Wt. %    | Cumul. wt. % |
| -1/4-6    | 62.05      | 62.05        | 53.73    | 53.73        | 51.55    | 51.55        | 57.33    | 57.33        | 53.71    | 53.71        | 53.97    | 53.97        | 52.86    | 52.86        | 62.38    | 62.38        |
| -6-8      | 18.01      | 80.06        | 18.29    | 72.02        | 19.42    | 70.97        | 17.57    | 74.90        | 17.68    | 71.39        | 18.19    | 72.16        | 18.16    | 71.02        | 14.60    | 76.98        |
| -8-10     | 10.32      | 90.38        | 11.16    | 83.18        | 11.92    | 82.89        | 10.66    | 85.56        | 11.35    | 82.74        | 11.14    | 83.30        | 11.41    | 82.43        | 9.41     | 86.39        |
| -10-14    | 6.81       | 97.19        | 9.44     | 92.62        | 9.82     | 92.71        | 8.11     | 93.67        | 9.06     | 91.80        | 8.91     | 92.21        | 9.31     | 91.74        | 7.05     | 93.44        |
| -14-16    | 1.76       | 98.95        | 3.91     | 96.53        | 3.64     | 96.35        | 3.22     | 96.89        | 3.71     | 95.51        | 3.52     | 95.73        | 3.96     | 95.70        | 2.72     | 96.16        |
| -16-20    | 0.65       | 99.60        | 2.07     | 98.60        | 2.21     | 98.56        | 2.00     | 98.89        | 1.97     | 97.48        | 1.99     | 97.72        | 2.10     | 97.80        | 1.11     | 97.27        |
| -20-28    | 0.21       | 99.81        | 0.46     | 99.06        | 0.44     | 99.00        | 0.44     | 99.33        | 0.66     | 98.14        | 0.59     | 98.31        | 0.58     | 98.38        | 0.99     | 98.26        |
| -28-35    | 0.10       | 99.91        | 0.23     | 99.29        | 0.17     | 99.17        | 0.11     | 99.44        | 0.22     | 98.36        | 1.99     | 98.54        | 0.35     | 98.73        | 0.50     | 98.76        |
| -35-48    | 0.01       | 99.92        | 0.35     | 99.64        | 0.33     | 99.50        | 0.22     | 99.66        | 0.76     | 99.12        | 0.59     | 99.13        | 0.47     | 99.20        | 0.50     | 99.26        |
| -48-65    | 0.01       | 99.93        | 0.12     | 99.76        | 0.22     | 99.72        | 0.11     | 99.77        | 0.22     | 99.34        | 0.35     | 99.48        | 0.34     | 99.55        | 0.25     | 99.51        |
| -65-100   | 0.01       | 99.94        | 0.12     | 99.88        | 0.11     | 99.83        | 0.06     | 99.83        | 0.22     | 99.56        | 0.12     | 99.60        | 0.24     | 99.78        | 0.19     | 99.70        |
| -100-150  | 0.01       | 99.95        | 0.06     | 99.94        | 0.06     | 99.89        | 0.06     | 99.59        | 0.22     | 99.78        | 0.17     | 99.77        | 0.11     | 99.89        | 0.06     | 99.76        |
| -150      | 0.05       | 100.00       | 0.06     | 100.00       | 0.11     | 100.00       | 0.11     | 100.00       | 0.22     | 100.00       | 0.23     | 100.00       | 0.11     | 100.00       | 0.24     | 100.00       |

Table 5.—Size distribution of soda feldspar samples after calcination but prior to grinding

| Mesh size | Uncalcined |              | 1000° F. |              | 1300° F. |              | 1500° F. |              | 1650° F. |              | 1800° F. |              | 2000° F. |              | 2150° F. |              |
|-----------|------------|--------------|----------|--------------|----------|--------------|----------|--------------|----------|--------------|----------|--------------|----------|--------------|----------|--------------|
|           | Wt. %      | Cumul. wt. % | Wt. %    | Cumul. wt. % | Wt. %    | Cumul. wt. % | Wt. %    | Cumul. wt. % | Wt. %    | Cumul. wt. % | Wt. %    | Cumul. wt. % | Wt. %    | Cumul. wt. % | Wt. %    | Cumul. wt. % |
| -1/4-6M   | 54.80      | 54.80        | 54.11    | 54.11        | 47.42    | 47.42        | 44.14    | 44.14        | 47.48    | 47.48        | 44.96    | 44.96        | 48.71    | 48.71        | 48.71    | 48.71        |
| -6-8      | 18.22      | 73.02        | 17.92    | 72.03        | 18.59    | 68.01        | 18.08    | 63.12        | 18.20    | 65.68        | 18.05    | 63.01        | 18.06    | 67.37        | 67.37    | 67.37        |
| -8-10     | 12.15      | 85.17        | 11.73    | 83.76        | 13.32    | 79.33        | 13.88    | 77.00        | 12.57    | 78.25        | 14.11    | 77.12        | 13.05    | 80.42        | 80.42    | 80.42        |
| -10-14    | 8.76       | 93.93        | 9.21     | 92.97        | 10.84    | 90.17        | 12.19    | 89.19        | 10.75    | 89.00        | 11.48    | 88.60        | 10.31    | 90.73        | 90.73    | 90.73        |
| -14-16    | 3.39       | 97.32        | 3.85     | 96.82        | 4.65     | 94.82        | 5.66     | 94.75        | 4.80     | 93.80        | 4.92     | 93.52        | 4.55     | 95.28        | 95.28    | 95.28        |
| -16-20    | 1.69       | 99.01        | 1.68     | 98.50        | 2.79     | 97.61        | 2.62     | 97.37        | 2.65     | 96.45        | 2.95     | 96.47        | 2.28     | 97.56        | 97.56    | 97.56        |
| -20-28    | 0.28       | 99.29        | 0.50     | 99.00        | 0.46     | 98.07        | 0.61     | 97.98        | 0.99     | 97.44        | 0.50     | 96.97        | 0.91     | 98.47        | 98.47    | 98.47        |
| -28-35    | 0.28       | 99.57        | 0.34     | 99.34        | 0.62     | 98.69        | 0.08     | 99.06        | 0.99     | 98.43        | 1.31     | 98.28        | 0.68     | 99.15        | 99.15    | 99.15        |
| -35-48    | 0.01       | 99.58        | 0.08     | 99.42        | 0.39     | 99.08        | 0.02     | 99.08        | 0.01     | 98.44        | 0.08     | 98.36        | 0.01     | 99.16        | 99.16    | 99.16        |
| -48-65    | 0.14       | 99.72        | 0.25     | 99.67        | 0.46     | 99.54        | 0.61     | 99.69        | 0.82     | 99.26        | 0.82     | 99.18        | 0.46     | 99.62        | 99.62    | 99.62        |
| -65-100   | 0.07       | 99.79        | 0.08     | 99.75        | 0.15     | 99.69        | 0.08     | 99.77        | 0.33     | 99.58        | 0.33     | 99.51        | 0.15     | 99.77        | 99.77    | 99.77        |
| -100-150  | 0.07       | 99.86        | 0.08     | 99.83        | 0.08     | 99.77        | 0.08     | 99.85        | 0.17     | 99.76        | 0.16     | 99.67        | 0.08     | 99.85        | 99.85    | 99.85        |
| -150      | 0.14       | 100.00       | 0.17     | 100.00       | 0.23     | 100.00       | 0.15     | 100.00       | 0.24     | 100.00       | 0.33     | 100.00       | 0.15     | 100.00       | 100.00   | 100.00       |

Table 6.—Size distribution of potash feldspar samples after calcination but prior to grinding

| Mesh size | Uncalcined |              | 1000° F. |              | 1300° F. |              | 1500° F. |              | 1650° F. |              | 1800° F. |              | 2000° F. |              | 2150° F. |              |
|-----------|------------|--------------|----------|--------------|----------|--------------|----------|--------------|----------|--------------|----------|--------------|----------|--------------|----------|--------------|
|           | Wt. %      | Cumul. wt. % | Wt. %    | Cumul. wt. % | Wt. %    | Cumul. wt. % | Wt. %    | Cumul. wt. % | Wt. %    | Cumul. wt. % | Wt. %    | Cumul. wt. % | Wt. %    | Cumul. wt. % | Wt. %    | Cumul. wt. % |
| -1/4-6    | 52.71      | 52.71        | 48.91    | 48.91        | 49.67    | 49.67        | 47.53    | 47.53        | 46.31    | 46.31        | 48.94    | 48.94        | 50.27    | 50.27        | 50.01    | 50.01        |
| -6-8      | 18.33      | 71.04        | 19.11    | 68.02        | 19.36    | 69.03        | 18.71    | 66.24        | 19.14    | 65.45        | 18.63    | 67.57        | 18.85    | 69.12        | 18.63    | 68.64        |
| -8-10     | 11.57      | 82.61        | 13.27    | 81.29        | 12.44    | 81.47        | 12.55    | 78.79        | 13.64    | 79.09        | 12.46    | 80.03        | 12.22    | 81.34        | 12.63    | 81.27        |
| -10-14    | 9.49       | 92.10        | 10.34    | 91.63        | 10.14    | 91.61        | 11.39    | 90.18        | 10.78    | 88.87        | 10.66    | 90.69        | 9.89     | 91.23        | 9.94     | 91.21        |
| -14-16    | 3.71       | 95.81        | 3.93     | 95.56        | 4.33     | 95.99        | 4.88     | 95.06        | 4.84     | 94.71        | 4.38     | 95.07        | 9.55     | 4.24         | 95.45    | 95.45        |
| -16-20    | 2.50       | 98.31        | 3.04     | 98.60        | 2.30     | 98.29        | 2.79     | 97.85        | 2.58     | 97.65        | 2.58     | 97.62        | 2.09     | 97.62        | 2.17     | 97.62        |
| -20-28    | 0.65       | 98.96        | 0.67     | 99.27        | 0.92     | 99.21        | 0.93     | 98.78        | 1.10     | 98.67        | 0.67     | 98.32        | 0.72     | 98.34        | 98.34    | 98.34        |
| -28-35    | 0.22       | 99.18        | 0.22     | 99.49        | 0.17     | 99.35        | 0.23     | 99.01        | 0.11     | 98.78        | 0.56     | 98.88        | 0.47     | 98.79        | 0.52     | 98.86        |
| -35-48    | 0.22       | 99.40        | 0.17     | 99.66        | 0.11     | 99.49        | 0.29     | 99.30        | 0.50     | 99.28        | 0.45     | 99.33        | 0.47     | 99.26        | 0.52     | 99.33        |
| -48-65    | 0.11       | 99.51        | 0.11     | 99.77        | 0.23     | 99.72        | 0.34     | 99.64        | 0.28     | 99.56        | 0.22     | 99.55        | 0.23     | 99.49        | 0.21     | 99.59        |
| -65-100   | 0.16       | 99.67        | 0.06     | 99.83        | 0.11     | 99.83        | 0.12     | 99.76        | 0.11     | 99.67        | 0.17     | 99.72        | 0.17     | 99.68        | 0.21     | 99.80        |
| -100-150  | 0.11       | 99.78        | 0.06     | 99.89        | 0.06     | 99.89        | 0.12     | 99.88        | 0.11     | 99.78        | 0.06     | 99.78        | 0.23     | 99.89        | 0.10     | 99.90        |
| -150      | 0.22       | 100.00       | 0.11     | 100.00       | 0.11     | 100.00       | 0.12     | 100.00       | 0.22     | 100.00       | 0.22     | 100.00       | 0.11     | 100.00       | 0.10     | 100.00       |

Table 7.—Size distribution of quartz samples after calcination but prior to grinding

| Mesh size | Uncalcined |              | 1000° F. |              | 1300° F. |              | 1500° F. |              | 1650° F. |              | 1800° F. |              | 2000° F. |              | 2150° F. |              |
|-----------|------------|--------------|----------|--------------|----------|--------------|----------|--------------|----------|--------------|----------|--------------|----------|--------------|----------|--------------|
|           | Wt. %      | Cumul. wt. % | Wt. %    | Cumul. wt. % | Wt. %    | Cumul. wt. % | Wt. %    | Cumul. wt. % | Wt. %    | Cumul. wt. % | Wt. %    | Cumul. wt. % | Wt. %    | Cumul. wt. % | Wt. %    | Cumul. wt. % |
| -1/4-6    | 53.43      | 53.43        | 57.96    | 57.96        | 52.46    | 52.46        | 50.66    | 50.66        | 48.39    | 48.39        | 52.98    | 52.98        | 51.42    | 51.42        | 50.16    | 50.16        |
| -6-8      | 16.44      | 69.87        | 16.40    | 74.36        | 17.79    | 70.25        | 18.72    | 69.83        | 18.47    | 66.86        | 17.32    | 70.30        | 17.77    | 69.19        | 17.74    | 67.90        |
| -8-10     | 11.79      | 81.66        | 10.94    | 85.30        | 11.90    | 82.15        | 11.75    | 81.13        | 10.21    | 80.07        | 11.77    | 82.07        | 12.55    | 81.74        | 12.50    | 80.40        |
| -10-14    | 9.98       | 91.64        | 8.07     | 93.37        | 9.71     | 91.86        | 10.27    | 91.40        | 11.10    | 91.17        | 9.96     | 92.03        | 9.99     | 91.73        | 10.57    | 90.97        |
| -14-16    | 4.08       | 95.72        | 3.28     | 96.65        | 4.27     | 96.13        | 4.45     | 95.85        | 4.67     | 95.84        | 4.07     | 96.10        | 4.22     | 95.95        | 4.32     | 95.29        |
| -16-20    | 2.77       | 98.49        | 1.78     | 98.43        | 2.31     | 98.44        | 2.62     | 98.47        | 2.80     | 98.64        | 2.04     | 98.14        | 2.33     | 98.28        | 2.61     | 97.90        |
| -20-28    | 0.56       | 99.05        | 0.41     | 98.84        | 0.69     | 99.13        | 0.68     | 99.15        | 0.82     | 99.46        | 1.02     | 99.16        | 0.89     | 99.17        | 0.91     | 98.81        |
| -28-35    | 0.34       | 99.39        | 0.27     | 99.11        | 0.12     | 99.25        | 0.29     | 99.44        | 0.12     | 99.58        | 0.23     | 99.39        | 0.33     | 99.50        | 0.34     | 99.18        |
| -35-48    | 0.22       | 99.61        | 0.41     | 99.52        | 0.12     | 99.37        | 0.17     | 99.61        | 0.18     | 99.76        | 0.11     | 99.50        | 0.11     | 99.61        | 0.34     | 99.49        |
| -48-65    | 0.11       | 99.72        | 0.14     | 99.66        | 0.23     | 99.60        | 0.11     | 99.72        | 0.12     | 99.88        | 0.11     | 99.61        | 0.11     | 99.72        | 0.23     | 99.72        |
| -65-100   | 0.11       | 99.83        | 0.07     | 99.73        | 0.11     | 99.71        | 0.11     | 99.83        | 0.06     | 99.94        | 0.11     | 99.72        | 0.11     | 99.83        | 0.11     | 99.83        |
| -100-150  | 0.06       | 99.89        | 0.14     | 99.87        | 0.06     | 99.77        | 0.06     | 99.89        | 0.06     | 100.00       | 0.11     | 99.83        | 0.11     | 99.94        | 0.11     | 99.94        |
| -150      | 0.11       | 100.00       | 0.13     | 100.00       | 0.23     | 100.00       | 0.11     | 100.00       | 0.17     | 100.00       | 0.06     | 100.00       | 0.06     | 100.00       | 0.06     | 100.00       |

This is also shown by Figure 4, in which the percentage of plus 16-mesh material is plotted against temperature for the calcined and uncalcined samples. From Figure 4 the greatest variation noted for any sample is about four per cent. For example, the uncalcined aplite sample contained 98.9 per cent of material between 1/4 inch and 16 mesh in size, and in the sample calcined at 1800° Fahrenheit this dropped to only 95.7 per cent. The disintegration caused by calcination is insignificant.

From the standpoint of use in ceramic ware, especially in the manufacture of glass, the most desirable size distribution of the ground aplite is one in which the maximum percentage is between 16 and 100 mesh. Tables 8, 9, 10 and 11, which follow, give the size distribution of the grindability products calcined and uncalcined for aplite, soda feldspar, potash feldspar and quartz, respectively.

Table 8.—Size distribution of aplite grindability products, calcined and uncalcined

| Mesh size | Uncalcined |              | 1000° F. |              | 1300° F. |              | 1500° F. |              | 1650° F. |              | 1800° F. |              | 2000° F. |              | 2150° F. |              |
|-----------|------------|--------------|----------|--------------|----------|--------------|----------|--------------|----------|--------------|----------|--------------|----------|--------------|----------|--------------|
|           | Wt. %      | Cumul. wt. % | Wt. %    | Cumul. wt. % | Wt. %    | Cumul. wt. % | Wt. %    | Cumul. wt. % | Wt. %    | Cumul. wt. % | Wt. %    | Cumul. wt. % | Wt. %    | Cumul. wt. % | Wt. %    | Cumul. wt. % |
| -16-28    | 12.2       | 12.2         | 10       | 10           | 14.9     | 14.9         | 17.2     | 17.2         | 30.6     | 30.6         | 28.3     | 28.3         | 27.5     | 27.5         | 23.7     | 23.7         |
| -28-35    | 9.6        | 21.8         | 14.2     | 24.2         | 19.1     | 34.0         | 14.6     | 31.8         | 19.4     | 50.0         | 16.9     | 45.2         | 20.3     | 47.8         | 20.1     | 43.8         |
| -35-48    | 11.2       | 33.0         | 13.1     | 37.3         | 3.0      | 37.0         | 15.3     | 47.1         | 6.7      | 56.7         | 10.9     | 55.1         | 8.7      | 56.5         | 17.8     | 61.6         |
| -48-65    |            |              |          |              |          |              |          |              |          |              |          |              |          |              |          |              |

Table 9.—Size distribution of soda feldspar grindability products, calcined and uncalcined

| Mesh size | Uncalcined |              | 1000° F. |              | 1500° F. |              | 1650° F. |              | 1800° F. |              | 2000° F. |              | 2150° F. |              |
|-----------|------------|--------------|----------|--------------|----------|--------------|----------|--------------|----------|--------------|----------|--------------|----------|--------------|
|           | Wt. %      | Cumul. wt. % | Wt. %    | Cumul. wt. % | Wt. %    | Cumul. wt. % | Wt. %    | Cumul. wt. % | Wt. %    | Cumul. wt. % | Wt. %    | Cumul. wt. % | Wt. %    | Cumul. wt. % |
| -16-28    | 14.7       | 14.7         | 16.1     | 16.1         | 22.1     | 22.1         | 26.6     | 26.6         | 28.1     | 28.1         | 34.3     | 34.3         | 29.0     | 29.0         |
| -28-35    | 16.4       | 31.1         | 11.1     | 27.2         | 14.9     | 37.0         | 12.2     | 38.8         | 20.4     | 48.5         | 11.8     | 46.1         | 11.3     | 40.3         |
| -35-48    | 17.6       | 48.7         | 22.6     | 49.8         | 21.7     | 58.7         | 26.0     | 64.8         | 14.9     | 63.4         | 19.9     | 66.0         | 22.6     | 62.9         |
| -48-65    | 16.0       | 64.7         | 15.6     | 65.4         | 14.3     | 73.0         | 12.5     | 77.3         | 13.9     | 77.3         | 11.4     | 77.4         | 12.3     | 75.2         |
| -65-100   | 9.0        | 73.7         | 8.9      | 74.3         | 7.7      | 80.7         | 6.9      | 84.2         | 7.2      | 84.5         | 7.1      | 84.5         | 7.4      | 82.6         |
| -100-200  | 10.9       | 84.6         | 11.1     | 85.4         | 8.1      | 88.8         | 7.2      | 91.4         | 7.2      | 91.7         | 7.4      | 91.9         | 7.7      | 90.3         |
| -200      | 15.4       | 100.0        | 14.6     | 100.0        | 11.2     | 100.0        | 8.6      | 100.0        | 8.3      | 100.0        | 8.1      | 100.0        | 9.7      | 100.0        |

Table 10.—Size distribution of potash feldspar grindability products, calcined and uncalcined

| Mesh size | Uncalcined |              | 1000° F. |              | 1300° F. |              | 1500° F. |              | 1650° F. |              | 1800° F. |              | 2000° F. |              | 2150° F. |              |
|-----------|------------|--------------|----------|--------------|----------|--------------|----------|--------------|----------|--------------|----------|--------------|----------|--------------|----------|--------------|
|           | Wt. %      | Cumul. wt. % | Wt. %    | Cumul. wt. % | Wt. %    | Cumul. wt. % | Wt. %    | Cumul. wt. % | Wt. %    | Cumul. wt. % | Wt. %    | Cumul. wt. % | Wt. %    | Cumul. wt. % | Wt. %    | Cumul. wt. % |
| -16-28    | 19.0       | 19.0         | 18.6     | 18.6         | 18.3     | 20.0         | 20.0     | 21.2         | 21.2     | 27.5         | 27.5     | 22.5         | 22.5     | 23.9         | 23.9     |              |
| -28-35    | 19.0       | 38.0         | 21.9     | 40.5         | 15.1     | 33.4         | 13.1     | 33.1         | 19.6     | 40.8         | 14.1     | 41.6         | 17.1     | 39.6         | 14.6     | 38.5         |
| -35-48    | 11.3       | 49.3         | 6.8      | 47.3         | 11.4     | 44.8         | 12.8     | 45.9         | 18.6     | 59.4         | 8.5      | 50.1         | 20.7     | 60.3         | 18.6     | 57.1         |
| -48-65    | 14.1       | 63.4         | 16.7     | 64.0         | 20.6     | 65.4         | 21.2     | 67.1         | 10.7     | 70.1         | 21.6     | 71.7         | 11.7     | 72.0         | 14.6     | 71.7         |
| -65-100   | 9.0        | 72.4         | 9.0      | 73.0         | 8.8      | 74.2         | 8.8      | 75.9         | 6.6      | 76.7         | 7.8      | 79.5         | 8.0      | 80.0         | 8.3      | 80.0         |
| -100-200  | 10.9       | 83.3         | 10.9     | 83.9         | 10.7     | 84.9         | 10.0     | 85.9         | 9.7      | 86.4         | 8.8      | 88.3         | 8.7      | 88.7         | 9.0      | 89.0         |
| -200      | 16.7       | 100.0        | 16.1     | 100.0        | 15.1     | 100.0        | 14.1     | 100.0        | 13.6     | 100.0        | 11.7     | 100.0        | 11.3     | 100.0        | 11.0     | 100.0        |

Table 11.—Size distribution of quartz grindability products, calcined and uncalcined

| Mesh size | Uncalcined |              | 1000° F. |              | 1300° F. |              | 1500° F. |              | 1650° F. |              | 1800° F. |              | 2000° F. |              | 2150° F. |              |
|-----------|------------|--------------|----------|--------------|----------|--------------|----------|--------------|----------|--------------|----------|--------------|----------|--------------|----------|--------------|
|           | Wt. %      | Cumul. wt. % | Wt. %    | Cumul. wt. % | Wt. %    | Cumul. wt. % | Wt. %    | Cumul. wt. % | Wt. %    | Cumul. wt. % | Wt. %    | Cumul. wt. % | Wt. %    | Cumul. wt. % | Wt. %    | Cumul. wt. % |
| -16-28    | 17.6       | 17.6         | 18.1     | 18.1         | 26.5     | 26.5         | 25.6     | 25.6         | 24.8     | 24.8         | 24.5     | 24.5         | 25.3     | 25.3         | 34.4     | 34.4         |
| -28-35    | 13.4       | 31.0         | 11.3     | 29.4         | 12.2     | 38.7         | 13.9     | 39.5         | 16.0     | 40.8         | 14.3     | 38.8         | 13.4     | 38.7         | 14.2     | 48.6         |
| -35-48    | 8.7        | 39.7         | 12.2     | 41.6         | 8.1      | 46.8         | 8.2      | 47.7         | 5.5      | 46.3         | 10.2     | 49.0         | 11.6     | 50.3         | 6.9      | 55.5         |
| -48-65    | 22.1       | 61.8         | 18.4     | 60.9         | 19.6     | 66.4         | 20.7     | 68.4         | 22.5     | 68.8         | 19.3     | 68.3         | 19.2     | 69.5         | 18.0     | 73.5         |
| -65-100   | 10.5       | 72.3         | 10.4     | 70.4         | 9.3      | 75.7         | 9.3      | 77.7         | 9.1      | 77.9         | 9.3      | 77.6         | 9.0      | 78.5         | 6.6      | 80.1         |
| -100-200  | 12.5       | 84.8         | 13.0     | 83.4         | 11.2     | 86.9         | 10.6     | 88.3         | 10.4     | 88.3         | 10.6     | 88.2         | 10.2     | 88.7         | 9.8      | 89.9         |
| -200      | 15.2       | 100.0        | 16.6     | 100.0        | 13.1     | 100.0        | 11.7     | 100.0        | 11.7     | 100.0        | 11.8     | 100.0        | 11.3     | 100.0        | 10.1     | 100.0        |

Table 12, which follows, gives the percentage and relative percentage increase of minus 16 plus 100 mesh sizes for the various calcined and uncalcined samples.

Table 12.—Percentage and percentage change in size distribution of grindability products, calcined and uncalcined, of aplite, soda feldspar, potash feldspar, and quartz

| Material        | Calcination temperature, degrees F. | Per cent of -16-100-mesh material in ground product | -16-100-mesh material as per cent of uncalcined material |
|-----------------|-------------------------------------|-----------------------------------------------------|----------------------------------------------------------|
| Aplite          | (1)                                 | 55.1                                                | 100                                                      |
| Do              | 1,000                               | 59.8                                                | 108                                                      |
| Do              | 1,300                               | 70.2                                                | 127                                                      |
| Do              | 1,500                               | 69.0                                                | 123                                                      |
| Do              | 1,650                               | 79.9                                                | 145                                                      |
| Do              | 1,800                               | 80.0                                                | 145                                                      |
| Do              | 2,000                               | 81.3                                                | 148                                                      |
| Do              | 2,150                               | 80.2                                                | 146                                                      |
| Soda feldspar   | (1)                                 | 73.7                                                | 100                                                      |
| Do              | 1,000                               | 74.3                                                | 101                                                      |
| Do              | 1,500                               | 80.7                                                | 109                                                      |
| Do              | 1,650                               | 84.2                                                | 114                                                      |
| Do              | 1,800                               | 84.5                                                | 115                                                      |
| Do              | 2,000                               | 84.5                                                | 115                                                      |
| Do              | 2,150                               | 82.6                                                | 112                                                      |
| Potash feldspar | (1)                                 | 72.4                                                | 100                                                      |
| Do              | 1,000                               | 73.0                                                | 101                                                      |
| Do              | 1,300                               | 74.2                                                | 102                                                      |
| Do              | 1,500                               | 75.9                                                | 105                                                      |
| Do              | 1,650                               | 76.7                                                | 106                                                      |
| Do              | 1,800                               | 79.5                                                | 110                                                      |
| Do              | 2,000                               | 80.0                                                | 110                                                      |
| Do              | 2,150                               | 80.0                                                | 110                                                      |
| Quartz          | (1)                                 | 72.3                                                | 100                                                      |
| Do              | 1,000                               | 71.5                                                | 97                                                       |
| Do              | 1,300                               | 75.7                                                | 104                                                      |
| Do              | 1,500                               | 77.7                                                | 107                                                      |
| Do              | 1,650                               | 77.9                                                | 108                                                      |
| Do              | 1,800                               | 77.6                                                | 107                                                      |
| Do              | 2,000                               | 78.5                                                | 109                                                      |
| Do              | 2,150                               | 80.1                                                | 111                                                      |

Uncalcined.

Figures 5 and 6 give the same data presented in Table 12 but in graphical form.

From Figure 5, it is apparent that uncalcined aplite, when ground to pass 16 mesh, contains the smallest percentage of the desired size, but that as the temperature of calcination increased to the critical range, the percentages of the desired sizes increased rapidly.

In Figure 6, the quantity of minus 16- plus 100-mesh material in the uncalcined samples is taken as 100 per cent, and the increase of this size in the calcined products is expressed in terms of the uncalcined value. This figure shows that the aplite has an increase of approximately 145 per cent in the critical range between 1650° and 2000° Fahrenheit. Soda feldspar, which next to aplite shows the greatest improvement, is increased to 110 per cent.

The data in Figure 6 again substantiates the opinion that soda feldspar, potash feldspar, and quartz cannot account for the increased grindability nor for the improved size distribution of the calcined samples of aplite.

#### Examination under the microscope

The behavior of aplite samples prior to and after calcination can also be verified by what is observed in thin sections of them under the polarizing microscope. To assist in presenting the correct picture, all of the photomicrographs reproduced in Figures 7 to 16 were made at a common magnification of 10 diameters.

In Figure 2, a grindability index of 2.1 was obtained for uncalcined aplite. Photomicrographs of this uncalcined sample are shown in Figures 7 and 8. These prints suggest why the aplite is hard to grind in an uncalcined state.

Under the polarizing microscope, it is apparent that the toughness of aplite may be accounted for by its massive crystalline structure and the absence of cleavage or other natural fracture planes. The photomicrograph reproduced in Figure 7, which is the same field as that reproduced in Figure 8 except that it was photographed without crossed nicols, shows this clearly in that the grain boundaries are almost extinct. Even at 340 magnifications only a very few fractures at the grain boundaries are noticeable and their width does not exceed two microns. Consequently, combining the knowledge of the hardness of the minerals present in aplite and the physical structure of aplite, it is understandable why the uncalcined aplite is difficult to grind.

Figures 9, 10, 11, 12, 13, 14, 15 and 16 present photomicrographs of the calcined aplite samples. Those calcined to temperatures of 1000, 1300 and 1500° Fahrenheit have an appearance similar to the uncalcined sample and nearly the same grindabilities. The samples calcined at 1650, 1800 and 2000° Fahrenheit show the presence of numerous fissures and cracks throughout the grains and along the grain boundaries. The boundary fissures are the most pronounced, and in the main, vary from 15 to 180 microns in width but some as wide as 300 microns were seen. The photomicrographs of the specimen calcined at 1650° Fahrenheit show the coarse preferential fissuring around the grains and is probably more typical than the photomicrographs of the sections calcined to 1800 and 2000° Fahrenheit which show the finer fissuring through the large grains of feldspar present in the aplite rock.

The extensive fissuring just cited for the calcination range 1650 to 2000° Fahrenheit indicates that the expansion was great and agrees with the dilatometer data presented in Figure 1 and the grindability indices plotted in Figure 2. The fissuring displayed in the aplite section calcined at 2150° Fahrenheit is not so pronounced and sharp as in the photomicrographs just discussed. The reason is best illustrated by the photomicrograph of the same field without crossed nicols which shows that most of the black lines are isotropic glass and not fissures. Recall that at this temperature the aplite became soft during calcination. Thus the fissures opened up by calcining in the temperature range 1650 to 2000° Fahrenheit are filled with glass when the material is further calcined to 2150° Fahrenheit. This accounts for the rapid drop in grindability at this temperature.

The photomicrographs explain the percentage change in size distribution caused by calcination which is also illustrated by Figure 6. The reason for the marked increase in minus 16 plus 100-mesh sizes for calcined aplite is that the fissuring caused by calcination is preferentially at the grain boundaries and the average grain size of aplite is 28-mesh. Uncalcined aplite contains no fissures to speak of.

#### Specific gravity determinations

In order to express quantitatively the magnitude of expansion caused by calcination, specific

gravity determinations were made. 100 minus  $\frac{1}{4}$  inch plus 6-mesh particles of each material were used and the determinations were made by desliming the solids in water, weighing in water, drying and weighing in air. Table 13 shows the data for uncalcined and 1800° Fahrenheit calcined samples. The aplite is the only sample displaying noticeably a change in specific gravity indicating expansion, which again verifies the dilatation and grindability data.

Table 13.—Specific gravities of calcined and uncalcined samples of aplite, soda feldspar, potash feldspar, and quartz

| Material             | Specific gravities |                      |
|----------------------|--------------------|----------------------|
|                      | Uncalcined         | Calcined at 1800° F. |
| Aplite.....          | 2.72               | 2.65                 |
| Soda feldspar.....   | 2.59               | 2.62                 |
| Potash feldspar..... | 2.58               | 2.58                 |
| Quartz.....          | 2.65               | 2.64                 |

#### Water quenching

As previously indicated, it is desirable to water-quench the aplite immediately after calcining. This results in greater thermal cracking and fracture of the aplite than when it is air-dried as in the previously discussed tests. In order to determine the effect of water-quenching after calcining, the following tests were made.

I took lumps of aplite, from two to three inches in diameter, and calcined the aplite at a temperature of about 1750° F. for a period of 30 minutes. Part of these lumps were then quenched in water and the other part was cooled in air. I then selected samples of the untreated aplite, samples of the treated and water quenched aplite and samples of the treated and air-cooled aplite and made crushing tests on these various samples. Great difficulty was encountered in crushing the untreated aplite. On the other hand, the treated and air-cooled aplite crushed easily and the treated and water quenched aplite even more easily.

In further tests relative to this invention, samples of the untreated aplite and samples of aplite treated in the manner indicated above and water-quenched were ground in such a manner that all particles would pass through a 16-mesh screen. It was found that in the case of the untreated ground aplite 38% of the ground material passed through a 200-mesh screen, or in other words, 38% of the material was in the form of excessive fines. On the other hand, in the case of the treated water-quenched aplite, only 5% of the ground material passed through a 200-mesh screen. This, obviously, definitely indicates that the production of fines during grinding is reduced to a minimum by the heat-treating and water-quenching operations.

Other tests were made to show the advantages of water-quenching over air-drying. The results obtained from these tests are indicated in Table 14.

Table 14.—Capacities obtained when dry grinding differently treated aplite in a rod mill under standard conditions

| Test conditions                                                                  | Weight per cent of original feed ground to minus 20-mesh | Weight per cent of -20-48M in ground product | Weight per cent of -48-100M in ground product | Weight per cent of -100-200M in ground product | Weight per cent of -200M in ground product |
|----------------------------------------------------------------------------------|----------------------------------------------------------|----------------------------------------------|-----------------------------------------------|------------------------------------------------|--------------------------------------------|
| Aplite calcined at 1800° F. for one-half hour, water quenched, and dry ground... | 75.2                                                     | 45.7                                         | 24.9                                          | 12.8                                           | 16.6                                       |
| Aplite calcined at 1800° F. for one-half hour, air cooled, and dry ground.....   | 50.1                                                     | 51.9                                         | 20.8                                          | 11.1                                           | 16.2                                       |

These tests definitely proved that water-quenching of the aplite after calcining is desirable.

#### Conclusion

It will be apparent from the above description that I have provided a process of treating aplite which has a number of advantages. These advantages may be summarized as follows:

1. Calcining aplite between the temperatures of 1000 and 2150° Fahrenheit improves its grindability, but the most effective and preferred range of calcining temperatures is between 1650 and 2000° Fahrenheit.

2. Calcining aplite within the preferred range increases its grindability to minus 16-mesh, 500 per cent and improves the desirable screen size composition of the ground product, minus 16 plus 100-mesh, by 150 per cent.

3. On being heated from 1650 to 1800° Fahrenheit, aplite passes through a transition point and permanent deformation takes place. The deformation is one of expansion and is characterized by the formation of large fissures along the grain boundaries and to a lesser extent across the mineral constituents of aplite.

4. The tests show that the results obtained by calcining aplite within its critical temperature range are caused by properties characteristic of aplite and not accountable for by soda feldspar, potash feldspar and quartz.

5. Water-quenching the aplite after calcining will increase its grindability further beyond that produced by air-quenching and will result in the

production of a greater amount of material of the proper screen size.

6. Calcining and grinding the aplite in the manner described will facilitate acid leaching to reduce the iron content in the manner described in Brenner and Dubble Patent No. 2,304,440, and will also facilitate magnetic separation.

Various other advantages will be apparent.

Having thus described my invention, what I claim is:

1. The method of treating aplite to reduce it to a grain size suitable for use in ceramic ware or for similar purposes, which comprises calcining 25 lumps of the aplite at a temperature sufficient to cause permanent expansion thereof, said temperature ranging from 1650° Fahrenheit to 2000° Fahrenheit, and then grinding the calcined lump aplite to a size such that all the ground material 30 will pass through a 16-mesh screen while having approximately 80 per cent of the total weight of the ground material greater than 100 mesh.

2. The method of treating aplite to obtain a product having a maximum particle size of -16 35 mesh and having more than approximately 80 per cent of the total weight greater than 100 mesh, said method comprising heating the aplite to a temperature between 1650° F. and 2150° F., cooling, and grinding so that substantially all of the said aplite will pass through a -16 mesh screen while having approximately 80 per cent of the total weight of the ground material greater than 100 mesh.

RALPH F. BRENNER.

CERTIFICATE OF CORRECTION.

Patent No. 2,387,561.

October 23, 1945.

RALPH F. BRENNER.

It is hereby certified that error appears in the printed specification of the above numbered patent requiring correction as follows: Page 5, Table 8, third column thereof, for the numeral "42,2" read --45.2--; and that the said Letters Patent should be read with this correction therein that the same may conform to the record of the case in the Patent Office.

Signed and sealed this 29th day of January, A. D. 1946.

Leslie Frazer

(Seal)

First Assistant Commissioner of Patents.